# EUROPEAN PATENT SPECIFICATION

(11) **EP 2 072 946 B1**
(45) Date of publication and mention of the grant of the patent: **06.04.2011**
(21) Application number: 07123506.3
(22) Date of filing: 18.12.2007
(51) Int. Cl.: F42B 12/76

(54) **Improved warhead casing**
Verbessertes Gehäuse für einen Gefechtskopf
Boîtier amélioré de charge militaire

(43) Date of publication of application: 24.06.2009
(73) Proprietor: SAAB AB, 581 88 Linköping (SE)
(72) Inventor: Ohlsson, Hans-Göran, 691 53 Karlskoga (SE); Karlsson, Geron, 691 41 Karlskoga (SE)
(74) Representative: Börlin, Maria

(56) References cited:
- EP-A- 0 392 084
- EP-A- 0 734 842
- US-A1- 2005 235 862

## Description

The present invention relates to a casing for a warhead or a warhead module.

### Prior art

Warheads used for various weapons systems typically comprise warhead casings manufactured from aluminium or steel. These materials are chosen for the casings since they need to be strong and have sufficiently low weight. However, such warheads have the disadvantage that they are likely to cause collateral damage, due to splinter from the warhead casing.

Attempts have been made to find alternative materials for warhead casings. In US 5000093 A, which forms a starting point for independent claim 1, a warhead casing is described which is made by isostatically pressing a mixture of magnesium and aluminium powder into a preform and then sintering the preform. This method may be suitable for simple warhead configurations, whereas more complicated configurations require additional machining after sintering. DE 10208228 describes a rotation symmetrical grenade having a casing of porous aluminium.

US 2005/0235862 A1 describes warhead structures fabricated by using high energy density technology. The warhead structures are made of metals.

There is a desire to avoid collateral damage, and thus there is a need to provide a warhead casing that fulfils the requirements set on warhead casings regarding weight and strength, but which does not cause collateral damage.

### Summary of the invention

According to the present invention a warhead casing having the features of independent claim 1 is provided. A laser sintered warhead casing presents several advantages over the casings previously available. It is splinter proof, whereby collateral damage can be avoided, and it can be made in one piece as opposed to steel or aluminium metal casings which have to be manufactured in separate components which are finally assembled. Moreover, laser sintering of the warhead casing allows for more complex geometries than have previously been possible to obtain for warheads in a simple way.

The laser sintered material has a density that is sufficiently low, for use in a warhead casing, and the weight is lower than the weight of aluminium alloys, which have a density of 2,7-2,8 g/cm³.

### Brief description of the drawings

Figures 1-3 illustrate examples of different geometries for warhead casings.

### Detailed description of the invention

By manufacturing casings for warheads or warhead modules by selective laser sintering technique, a decrease in the weight of such components can be achieved, since laser sintered materials have lower density than solid materials.

Warhead casings are-typically rotationally symmetrical. However, due to the flexibility of laser sintering other geometries may be contemplated, so that the warhead casing may be unsymmetrical. The warhead casing has the form of a hollow container, which is typically provided with an opening for filling of explosive. The hollow container comprises one or more wall surface portions, which constitute the container wall. The wall surface portions may be flat or curved. The filling opening may be a cylindrical portion protruding from one of the wall surfaces.

As an example, the warhead casing may have an unsymmetrical geometry, defining a hollow body, having a flat upper wall and a somewhat curved lower wall opposite the upper wall, a rear flat wall and a front flat wall. The height of the hollow body is larger at the rear end, than at the front end. An opening for filling with explosives is arranged in the flat upper surface, close to the rear wall.

Figures 1-3 illustrate examples of different geometries for warhead casings. The warhead casing of Fig. 1 has an opening **1** for filling of explosive **2,** arranged in a flat upper wall **3,** from which three flat wall surfaces **4a, 4b, 4c** extend sloping slightly downwards. All these three flat wall surfaces are connected to a rounded wall surface **5** which constitutes the wall opposite the filling opening. In one of the flat surfaces **4b** and partly in the rounded wall surface is provided an indentation **6.**

Fig. 2 illustrates a geometry in which the filling opening **7** extends from a circular surface **8,** from which a rounded surface **9** extends downwardly in the form of a truncated cone. At the lower end of the lower wide end of the conical surface flat surfaces **10** extend. Three indentations **11** are provided in these flat surfaces. The bottom surface **12** opposite to the filling opening is flat.

The geometry illustrated in Fig. 3 has the form of an elongated container having the filling opening (not shown) arranged in a side wall at the end of a truncated cone. The longitudinal cross-sectional area at the centre of the container (the cross-section of which is shown in Fig. 3) is larger than the cross-sectional area at each side of the container. Indentations **13** are provided in the central portion of the container wall surface.

Laser sintering has hitherto primarily been used for manufacturing of prototypes for this application. The strength of laser sintered material is not sufficient without reinforcement for extremely high launch forces, but good enough for moderate launch forces. Laser sintering allows for shaping of_complex geometries in one piece, and normally no further machining is required, except possibly clearing of screw threads. An example of the laser sintering technology is described in EP0734842A1.

Laser sintering technology utilizes a model of the object to be manufactured, such as a CAD model. A laser beam is moved layer by layer over a powder bed of fine particles in accordance with the model. The laser beam locally heats the powder to the melting point, without the temperature exceeding the melting point, and the powder grains are thereby sintered together. An article having the same geometry as the model is thus built up layer by layer. On cooling the finished model is broken out of the "cake" of unsintered powder and brushed clean. Selective laser sintering allows generating complex three dimensional objects by consolidating successive layers of powder material on top of each other.

The powder blend for manufacture of the warhead casing of the present invention comprises metal particles and particles of a binding component. The powder blend may comprise fine grained aluminium powder and polymer powder.

The preferred average grain size of the aluminium powder is 10-90 µm, more preferably 30-70 µm, and most preferably 45-55 µm.

The polymer used is preferably a polyamide, such as nylon-powder, which may have a particle diameter of 0,05-0,2 mm. The polyamide improves the binding of the particles to each other. An example of a laser sintered material suitable for warhead casings or warhead modules is Alumide^{®}, available from EOS Gmbh, Germany. Alumide^{®} is made up of 50% fine aluminium powder suspended in polyamide (Nylon 12).

An alternative polymer may be polychlorotrifluoroethylene (PCTFE) which is fluorocarbon based polymer. PCTFE may be favourable in view of the enhanced combustion properties.

An alternative to aluminium powder in the laser sintered material may be magnesium powder.

The surfaces of the laser sintered parts can be finished by grinding, polishing, or coating. An additional advantage is that low tool-wear machining is possible, e.g. milling, drilling, or tuning.

Subsequent to forming, the laser sintered warhead casing is filled with a desired explosive composition. The explosive composition preferably includes aluminium powder. Aluminium plays an important role in both the shock response and energy release rates of energetic materials.

When the explosive composition detonates, the aluminium powder of the explosive composition is dispersed and rapidly burns. At the same time the casing is disintegrated. As the warhead casing is made up of laser sintered aluminium and/or magnesium, the metal grains that the casing was made up of will participate in the explosive reaction and will thus contribute to the effect obtained.

The explosive composition used in the in the warhead may include aluminium powder in an amount of 15-50 % by weight of the total composition, which reacts with the air oxygen. Too high aluminium powder content doesn't serve any purpose, since the air oxygen available for reaction is limited. An aluminium powder content of approximately 19-21 % by weight, results in an explosive composition that is easy to handle and easy to fill in the warhead casing. The aluminium powder typically has an average particle size between 12 and 18 µm.

The explosive composition may be based on a nitroamine explosive, such as RDX (hexogen or cyclotrimethylene-trinitramine) or HMX (octogen or cyclotetramethylene-tetranitramine), and may in addition to aluminium powder also comprise a binder. The amount of nitroamine explosive (e.g. RDX) may be approximately 65% by weight of the explosive composition. The binder may be present in approximately 15% by weight.

The binder may comprise a binder agent (e.g. HTPB (hydroxyl-terminated polybutadiene)), plasticizer (e.g. DOA (dioctyl adipate)), surfactant (e.g. DHE (N,N-di-(2-hydroxyethyl)-4,4-dimethylhydantoin)), cure catalyst (e.g. triphenylbismuth) and curing agent (e.g. IDPI (isophorone diisocyanate)).
A specific example of a suitable explosive is PBXN-109, comprising 65% RDX, 15% HTPB (binder) and 20% Al.

As the laser sintered material is not completely impermeable, it may be necessary to provide the casing with a sealing lacquer coating before filling it with the explosive, in order to enhance the impermeability. The lacquer coating must be compatible with the explosive, to avoid undesired reactions. The lacquer may for example be an epoxy resin lacquer, such as RenLam^{®}, comprising resin and curing agent (e.g. RenLam LY 113/HY 97).

The laser sintered casing may also be reinforced by an outer lining of reinforced fibre type, e.g. carbon or Kevlar, to be able to withstand large launching forces.

The warhead casing thus manufactured will be splinter free, unless it is not provided with an additional metal casing.

As the explosive composition of the warhead detonates, the aluminium powder of the explosive composition will ignite and burn.

### Example

A test warhead casing was manufactured by laser sintering of Alumide^{®}. The test warhead was a cylindrical, hollow body with a material thickness of 4mm and a weight of 375 g, which was filled with 2 kg explosive composition PBXN-109. The warhead was lacquered with RenLam^{®}.

The test warhead casing was subjected to low temperature and high temperature tests. In each test the test warhead casing was placed in Weiss 1 climate chamber. Under a first period of time, the temperature in the climate chamber was changed from an initial temperature to a goal temperature. Under a second period of time the temperature in the climate chamber was maintained at the goal temperature, and under a third period of time the temperature in the climate chamber was changed from the-goal temperature to en end temperature.

After each test, the test warhead was examined for damages, by means of ocular inspection. No damages could be observed.

Temperatures and duration of time periods are displayed in Table 1 below.

**Table 1**

| | Initial temp (°C) | Goal temp. (°C) | Time to reach goal temp. (hours) | Time period maintained at end temp. (hours) | End temp. (°C) | Time to reach end temp. (hours) | Damages observed after test period (yes/no) |
|---|---|---|---|---|---|---|---|
| Low temperature test | +21 | -46 | 12 | 24 | +21 | 12 | no |
| High temperature test | +21 | +75 | 12 | 48 | +21 | 12 | no |

The test warhead was also subjected to a vibration test (STANAG 4242/APO-34). In this test the warhead was mounted on a fixture of a test equipment (vibrator system LDS 954, amplifier MPA 32, control system DACTRON Dual DSP) and was subjected to vibrations for two hours in each of three directions (x-, y-, and z-directions) in a temperature of approx. 20°C. The measuring equipment used was an accelerometer KISTLER ICP. Thereafter, the test casing was examined for damages. No damages could be observed.

Comparative calculations performed on warhead casing of steel and laser sintered Alumide^{®} show that the laser sintered Alumide^{®} casing should theoretically result in an increased over pressure of 28% in a volume of 40 m³.

## Claims

1. A casing for warhead components, **characterized in that** the casing is made up of a laser sintered material, wherein the laser sintered material comprises polymer particles and aluminium or magnesium powder.

2. The casing of claim 1, wherein said aluminium powder has an average grain size of 10-90, preferably 45-55 µm.

3. The casing of claim 1, wherein the polymer particles comprise a polyamide.

4. The casing of claim 1, wherein the polymer particles comprise a polychlorotrifluoroethylene.

5. The casing of any one of claims 1-4, wherein the casing is provided with a lacquer coating.

6. The casing of any one of claims 9-5, wherein the casing is provided with an outer lining of e.g. Kevlar.

7. A warhead comprising a casing as defined in claims 1-6.

8. The warhead of claim 7, wherein the casing is filled with a polymer bonded explosive composition (2) comprising a binder, and aluminium powder.

## Patentansprüche

1. Gehäuse für Gefechtskopfbauteile, **dadurch gekennzeichnet, dass** das Gehäuse aus einem lasergesinterten Material hergestellt ist, wobei das lasergesinterte Material Polymerpartikel und Aluminium- oder Magnesiumpulver umfasst.

2. Gehäuse nach Anspruch 1, bei dem das Aluminiumpulver eine durchschnittliche Korngröße von 10-90, bevorzugt 45-55µm aufweist.

3. Gehäuse nach Anspruch 1, bei dem die Polymerpartikel ein Polyamid umfassen.

4. Gehäuse nach Anspruch 1, bei dem die Polymerpartikel ein Polychlortrifluorethylen umfassen.

5. Gehäuse nach einem der Ansprüche 1-4, bei dem das Gehäuse mit einer Lackbeschichtung versehen ist.

6. Gehäuse nach einem der Ansprüche 1-5, bei dem das Gehäuse eine äußere Beschichtung aus beispielsweise Kevlar aufweist.

7. Gefechtskopf, umfassend ein Gehäuse nach einem der Ansprüche 1-6.

8. Gefechtskopf nach Anspruch 7, bei dem das Gehäuse mit einer polymergebundenen, explosiven Zusammensetzung (2), umfassend ein Bindemittel und Aluminiumpulver gefüllt ist.

## Revendications

1. Carter destiné à des composants d'ogive, **caractérisé en ce que** le carter est réalisé dans un matériau subissant un frittage laser, où le matériau subissant un frittage laser comprend des particules polymères et de la poudre d'aluminium ou de magnésium.

2. Carter selon la revendication 1, où ladite poudre d'aluminium présente une granulométrie moyenne de 10-90, de préférence de 45-55 µm.

3. Carter selon la revendication 1, où les particules polymères contiennent un polyamide.

4. Carter selon de la revendication 1, où les particules polymères contiennent un polychlorotrifluoroéthylène.

5. Carter selon l'une quelconque des revendications 1 à 4, où le carter comporte un revêtement de vernis.

6. Carter selon l'une quelconque des revendications 1 à 5, où le carter comporte un revêtement extérieur de kevlar, par exemple.

7. Ogive comprenant un carter tel que défini dans les revendications 1-6.

8. Ogive selon la revendication 7, où le carter est rempli d'un produit composé explosif (2) à liaison polymère et qui comprend un liant et de la poudre d'aluminium.
